

## UNITED STATES PATENT OFFICE

2,414,858

## TANNING OF PROTEINS

Paul B. Davidson, Wilkinsburg, Pa., assignor to  
Strathmore Paper Company, Springfield, Mass.,  
a corporation of Massachusetts

No Drawing. Application December 4, 1940,  
Serial No. 368,538

8 Claims. (Cl. 117—154)

1

This invention relates to the art of tanning water-dispersable proteins such as animal glues and casein, and particularly to the toughening and insolubilizing of sizings and other coatings as applied to paper and like materials.

It is common practice in the manufacture of certain types of paper to apply a surface treatment or sizing of animal glue or starch to the paper for the purpose of imparting to the paper certain characteristics such as strength, greater resistance to the penetration of liquids such as inks, erasure properties, increased durability and permanence, and stiffness. In some specialty papers, such as blue print paper, there are the added requirements of sufficient tensile strength and resistance to abrasion when the paper is wetted or soaked in water. This soaking in water is a necessary part of the developing of the exposed prints and is carried on with the paper under tension and the water is often applied under pressure.

A common prior way of sizing such paper is to pass the paper into a bath of animal glue and then between rolls that squeeze off the excess of glue. In the prior art, the glue is applied to the paper at a temperature of about 140° F. so that, due to its lower viscosity at this temperature, it will penetrate into the paper and produce a more or less complete saturation of the paper with the glue size. Aluminum sulphate (papermaker's alum) and formaldehyde have been added to the glue bath as tanning agents, for developing high wet tensile strength and resistance to abrasion when wet. This procedure has its undesirable features, such as the development of abnormally high viscosity of the glue, so that difficulty is encountered in the surface- or tub-sizing operation. To eliminate this difficulty, employment has been made of a process of omitting a tanning agent from the glue bath and then giving the freshly sized paper, before it has been dried, a separate treatment with a tanning agent. Formaldehyde has been used in such a treatment. There are various ways in which this may be accomplished: thus, a water solution of the formaldehyde may be sprayed onto the freshly sized and undried paper or the paper may be passed through a bath containing the water solution of this tanning agent and the excess squeezed off before the paper is dried; or the paper may be passed through a chamber filled with vaporized formaldehyde.

For some special types of paper, such as blue print paper, this method of glue sizing does not

produce the best results, particularly with respect to wet strength.

Further, there are serious disadvantages to the use of formaldehyde as a tanning agent, irrespective of the method by which it is applied. In the first place, a large part is driven off during the drying of the paper and, for this reason, an excess of the tanning agent must be originally applied so that satisfactory wet strength may be developed in the paper; and small variations in the drying of the paper cause varying quantities of the formaldehyde to be driven off, with a corresponding change in the tanning efficiency and in the strength characteristics of the product. Secondly, the accumulation of formaldehyde gas around open drying equipment for the paper may be so great that it produces irritating effects and disagreeable working conditions. Thirdly, paper that has been dried, apparently quite satisfactorily to remove water and the excess of formaldehyde, will often cause trouble when it is used due to the fact that there still remains in the paper an appreciable amount of formaldehyde; with such papers as blue print papers, where the paper is subjected to drying after the printing operation, the evolution of formaldehyde may then cause a disagreeable odor to develop.

An object of this invention, therefore, is to eliminate these undesirable conditions and other disadvantages by the use of a water-soluble, saturated, aliphatic dialdehydes as the tanning agent in paper manufacture. Dialdehydes are sometimes called dials. Glyoxal is the dialdehyde of ethylene glycol. It can be obtained in its monomeric form by heating the polymer with phosphorus pentoxide; but the polymerized glyoxal can be used as such and is the material referred to in the specific examples set forth hereinafter. In its solid form it is a colorless solid material containing about 25 percent of water of hydration, has no odor, does not volatilize like formaldehyde, and has a tanning efficiency at least equal to that of formaldehyde.

A great advantage in the use of a dialdehyde such as glyoxal as a tanning agent for glue size is that it does not volatilize in the paper driers. It thus follows that objectionable vapors are not evolved during manufacture or in the hands of the user of the paper. Its non-volatility from the paper allows the production of a greater tanning effect due to the fact that all of the tanning agent applied remains in the paper to react with the glue.

Another advantage in the use of glyoxal is that

it produces greater wet strength in the paper than can be obtained with formaldehyde under the same conditions. This is particularly true with respect to the resistance to abrasion when the paper is wet with water. Under some conditions, glyoxal has been found to produce wet rub values twice as great as are obtained with formaldehyde and under other conditions four times as great. This appears to be a peculiar effect of glyoxal in its reaction with proteins, for this same degree of improvement is not consistently found in the wet tensile strengths.

From a knowledge of the reaction of formaldehyde and proteins, it would logically appear that glyoxal tanning would depend, for its efficiency, upon the pH of the protein, which illustratively is animal glue. That is, formaldehyde reacts more rapidly and/or more completely with glue of high pH value (about 8.5) than with one of pH 7 and still more than with glue at a pH lower than the isoelectric point of the protein in the glue, as for example at a pH of 3.5. It has been found that this relationship between the pH of the glue and the tanning efficiency of glyoxal does not follow parallel to that of formaldehyde. Whereas formaldehyde produces decreasing strength with decreasing pH of the glue size, glyoxal produces wet strengths of the same magnitude substantially irrespective of the pH of the glue size. This is illustrated in the following table of results of experiments in which the same lot of paper was tub-sized with animal glue of varying pH and then passed through a bath of the tanning agent, made up to a 2 percent concentration, the excess of solution was squeezed off by passing the papers between rolls, and the paper then dried at a temperature of 95±5 degrees C.

Table I

Wet tensile strength with glue size of varying pH after a 24-hour aging period

| Tanning agent   | pH of glue size |      |      |      |      |      |      |      |
|-----------------|-----------------|------|------|------|------|------|------|------|
|                 | 2.4             | 3.45 | 4.57 | 4.7  | 5.17 | 5.67 | 7.06 | 8.5  |
| 2% formaldehyde | 1070            | 1190 | 1280 | 1320 | 1370 | 1110 | 1350 | 1370 |
| 3% glyoxal      | 1910            | 2000 | 2010 | 2110 | 2160 | 2160 | 2020 | 2040 |

Wet tensile values are expressed in grams per 15 mm. width of test strip.

If, for any reason, the wet strengths are insufficient to meet certain demands, it has been common practice to age the paper for an indefinite time to allow a slow further tanning of the glue by the formaldehyde to take place. This increase in wet strength with aging is more pronounced with glyoxal tanning of the glue size than with formaldehyde tanning. The wet tensile strength values in the following table, compared with those in the table above, will illustrate this point.

Table II

Wet tensile strength with glue of varying pH after a 6 day aging period

| Tanning agent   | pH of glue size |      |      |      |      |      |      |      |
|-----------------|-----------------|------|------|------|------|------|------|------|
|                 | 2.40            | 3.45 | 4.57 | 4.70 | 5.17 | 5.67 | 7.06 | 8.50 |
| 2% formaldehyde | 1110            | 1270 | 1320 | 1420 | 1400 | 1360 | 1340 | 1400 |
| 2% glyoxal      | 2120            | 2210 | 2100 | 2200 | 2410 | 2180 | 2210 | 2340 |

When a high pH glue solution is used, the uniformity of the desired properties also depends

upon the proper buffering of the glue size at the required pH values. A presently preferred buffering agent is borax, while magnesium oxide, magnesium carbonate and other combinations of materials as alkaline buffering agents that will maintain the pH of the glue within the limits of about 8 to 9.5, may be employed. The quantity to be employed depends upon the engine sizing efficiency; and this in turn depends upon the amount of papermaker's alum, since the leaching of alum from the paper renders the employment of such a buffer necessary. A further factor in determining the quantity is the amount of paper to be sized with a given quantity of the size, as this likewise influences the possible amount of leaching.

In the mill scale preparation of the glue size, the following formulas are typical. In each case, substantially 600 gallons of glue sizing solution was prepared.

## EXAMPLE I

High pH size (pH of 8.5)

|                                                 |         |     |
|-------------------------------------------------|---------|-----|
| (A) Animal glue (12.5% sol=110 M. P. viscosity) | lbs--   | 300 |
| Water                                           | gals--  | 250 |
| Sodium hydroxide                                | grams-- | 654 |
| Preservative (sodium ortho-phenyl phenate)      | kg--    | 28  |

The sodium hydroxide was dissolved in the water, to which the glue was added and allowed to soak and swell for two hours, with brief agitation from time to time, and then steam-cooked at 130 degrees to 140 degrees F. to completely disperse the glue.

|                |        |          |
|----------------|--------|----------|
| (B) Water      | gals-- | 100      |
| Buffer (borax) | lbs--  | 12 to 27 |

The hot glue dispersion (A) was then added, with stirring, to the solution B, and after thorough mixing was diluted to the desired Beaumé, giving 600 gallons of glue sizing solution. Twelve pounds of a suitable filler may be suspended in solution B, if desired.

The effect of mixing brings the system to about the proper temperature for sizing, i. e., between 90 degrees and 115 degrees F.

## EXAMPLE II

Low pH size (pH of 4.2)

|                                |          |      |
|--------------------------------|----------|------|
| Glue                           | lbs--    | 300  |
| Water                          | gals--   | 250  |
| Hydrochloric acid (36 percent) | liters-- | 6.25 |

The hot glue solution was made up as in Example I, and then stirred into 100 gallons of water, in which 12 lbs. of a suitable filler may be suspended. This cooled the glue below the temperature of any active hydrolysis; and the solution was then diluted to the desired Beaumé, and gave substantially 600 gallons of glue sizing solution at the desired temperature.

The quantity of glue can be adjusted in accordance with its properties for obtaining the desired concentration and Beaumé. The amount of alkali or acid added is sufficient to obtain the desired pH, between 3.5 and 9 or even higher being found effective: the specific pH value depends upon the ingredients and history of the paper being sized, and upon the desired viscosity of the glue solution at the temperature of employment. In preparing glue sizes of high pH, the alkali may be sodium, potassium or ammonium hydroxide, or another proper alkaline material: successful glue sizes have been prepared with tertiary amines. When the pH value is

high (above neutral), an alkaline buffering agent is introduced. When a low pH sizing solution is being prepared, the penetration of the alum of itself will lower the pH slightly and normally increase the viscosity of the glue; and this may be taken into account in determining the quantity of acidifying agent to be utilized. In some cases, it has been found desirable to add inert fillers to the size to improve certain surface properties of the paper. That is to say, if the paper is to be treated with a water-dispersed system, such as dextrose adhesives, or a solution such as blue print coating solutions, the presence of a proper filler often has desirable effects. In the case of blue print paper, for example, it has been found that titanium dioxide and/or bentonite improves the color produced in the final prints. Some fillers (such as calcium sulphate) cannot be used for this specific purpose, for they are not inert and react unfavorably with sensitizing chemicals.

The paper is sized with such a solution by passing the paper through it, and then passing it through a solution containing about 2 percent of glyoxal and between 0.02 and 0.5 percent of a wetting agent, and is then dried.

Between the application of the sizing solution and of the wetting agent, the paper may be aged if desired for the purpose of effecting a primary stabilization. A better product usually results when the paper is drawn through the solutions to produce a coating and treatment by a double-side dip.

The wetting agent is not invariably necessary, but is desirable for eliminating the last traces of white spots in blue prints. It has been discovered that not all wetting agents are of value in this process, but only those commonly known as neutral or cationic wetting agents serve the purpose. That is to say, a wetting agent is employed that is either classed colloidally as having no electrical charge or as being charged colloidally with a positive charge. A neutral wetting agent that has been found to be successful for this type of paper is a distearate of a highly polymerized glycol; other neutral long-chain fatty acid esters may be used. The cationic wetting agents comprise a class consisting of either condensation products of long chain fatty acids and ethanolamines or long carbon chain compounds that contain a tertiary amine group or a quaternary salt of such a tertiary amine. The term long chain fatty acids is applied to those which are water-insoluble, that is, which have 10 or more carbon atoms in the chain; and a corresponding length is used for the other designated long chain compounds. The presence of such wetting agents in the tanning agent solution facilitates the action of the tanning agent and produces higher wet strengths in the paper. It has been found experimentally, for example, that a solution containing 2 percent of glyoxal and 0.3 percent of a tertiary amine wetting agent, having a trade name of "Ninol," produced a five-fold improvement in wet rub over a paper sized with the same glue size but treated with 2 percent of formaldehyde.

It has been found that glyoxal and such wetting agents can be employed jointly, without loss of efficiency by either material.

It is presently preferred to maintain the proportion of glyoxal in the tanning solution between 0.5 and 2.0 percent. At the lower figure, the wet tensile strengths with paper aged for six

days is substantially the same as that tanned with 2% formaldehyde solution.

When the paper is being made for employment as a base for a blue print coating solution, it has been found in some instances that spoilage of the coated papers occurs at high relative humidities when a technical grade of glyoxal is employed; and for such cases it is recommended to employ the substances in purified condition.

10 Mixtures of formaldehyde and glyoxal can be used quite satisfactorily for the development of the necessary wet strengths in glue tub-sized papers. A mixture of 1 percent of formaldehyde and 1 percent of glyoxal produces wet tensile strengths intermediate between those obtained with either formaldehyde or glyoxal when used alone, provided that in the tanning treatment the paper is immersed in the solution of the tanning agents and the excess solution then squeezed off. If, however, the paper is not passed or immersed in the solution but passed directly through the nip of the squeeze rolls, one of which rolls is partially immersed in the solution of tanning agent for application to one side only, then the mixture of formaldehyde and glyoxal produces wet strengths higher than those obtained with either of these tanning agents used alone.

15 The behavior of glyoxal in reaction with animal and vegetable proteins may be seen from the following condensed table of results when animal glue, animal casein, and soybean protein (vegetable casein) have been employed in sizing paper:

### EXAMPLE III

|    | Tanning solution  | Animal glue | Casein | Soybean protein |
|----|-------------------|-------------|--------|-----------------|
|    |                   |             |        |                 |
| 40 | None              |             |        |                 |
|    | 2% formaldehyde   | 1020        | 860    | 930             |
|    | 2% glyoxal (pure) | 1510        | 1020   | 1070            |
| 45 | None              | 1700        | 1660   | 1730            |
|    | 2% formaldehyde   |             |        |                 |
|    | 2% glyoxal (pure) | 5           | 4      | 4               |
|    |                   | 17          | 8      | 7               |
|    |                   | 100+        | 100+   | 100+            |

50 Other water-soluble, saturated, aliphatic dials possess tanning action for animal and vegetable protein and are likewise lacking in physiological disadvantages, but they do not appear as efficient as glyoxal. That is to say, they do not produce as high wet tensile strengths when used in equivalent concentrations: for example, a 2 percent solution of succindialdehyde is about the same in effect as a 2 percent solution of formaldehyde, and a 6 percent solution of methyl glyoxal has essentially the same effect as a 2 percent formaldehyde solution.

55 It will be understood that this reaction of a suitable dialdehyde upon such proteins as animal glue and caseins may be employed for purposes other than paper sizing. It is obvious that the illustrative examples are not given as restrictions, but that the invention may be employed in many ways within the scope of the claims.

60 I claim:

65 1. The process of sizing paper and like material with an animal glue applied to a surface thereof, and having high wet tensile and wet rub strengths, which comprises passing the glue-sized paper through squeezing rolls with the deposited glue in contact with a rotating squeeze roll which is partially immersed in an aqueous solution containing substantially 1 percent each of formaldehyde and glyoxal.

2. A paper sheet having a wet tensile strength in excess of substantially 1940 grams per 15 millimeter width and having a high wet rub value, and being characterized in having thereon a sizing comprising the reaction product of animal glue with glyoxal.

3. The process of producing sized paper of high wet tensile and wet rub strengths for receiving the blueprint coatings, which comprises applying a water-dispersed animal glue solution to the surface thereof; thereafter subjecting the same to the action of an aqueous solution containing substantially 0.5 to 6 percent of a water-soluble saturated aliphatic dialdehyde selected from the group consisting of glyoxal, succindialdehyde and methyl glyoxal, in the presence of a water-soluble cationic wetting agent, said wetting agent being characterized in that it does not liberate an anion having active wetting properties in the ionized condition, and then subjecting the treated paper to aging.

4. The process of producing sized paper of high wet tensile and wet rub strengths for use as a base for blueprint papers, which comprises applying to the material a water-dispersed animal glue solution of pH of about 8 to 9.5 at a temperature of substantially 90 to 115 degrees F., said solution including an alkaline buffering agent, and thereafter subjecting the same to the action of an aqueous solution containing substantially 0.5 to 2 percent of polymerized glyoxal, in the presence of substantially 0.02 to 0.5 percent of a water-soluble cationic wetting agent.

5. The process of producing sized paper of high wet tensile and wet rub strengths, which comprises applying a water-dispersed animal glue solution having a pH between 3.5 and about 9 to the surfaces thereof, and thereafter subjecting the same to the action of an aqueous solution containing substantially 0.5 to 2 percent of glyoxal in the presence of a water-soluble wetting agent comprising a condensation product of a

water-insoluble long-chain fatty acid with ethanolamine, said product being characterized in that it does not liberate an anion having active wetting properties in its ionized condition.

6. A tanning solution for preparing blueprint papers having animal glue size thereon for thereby attaining uniform high wet tensile and wet rub strengths, comprising substantially 0.5 to 2.0 percent of polymerized glyoxal, and 0.02 to 0.5 percent of a water-soluble cationic wetting agent.

7. The process of producing sized paper of high wet tensile and wet rub strengths for receiving blueprint coatings, which comprises applying a water-dispersed animal glue solution to the surface thereof; thereafter subjecting the same to the action of an aqueous solution containing substantially 0.5 to 6 percent of a water-soluble saturated aliphatic dialdehyde selected from the group consisting of glyoxal, succindialdehyde and methyl glyoxal, in the presence of a long-chain carbon compound containing a tertiary amine and effective as a water-soluble cationic wetting agent, said wetting agent being characterized in that it does not liberate an anion having active wetting properties in the ionized condition, and then subjecting the treated paper to aging.

8. The process of producing sized paper of high wet tensile and wet rub strengths for use as a base for blueprint papers, which comprises applying to the material a water-dispersed animal glue solution of pH of about 8 to 9.5 at a temperature of substantially 90 to 115 degrees F., said solution including an alkaline buffering agent, and thereafter subjecting the same to the action of an aqueous solution containing substantially 0.5 to 2 percent of polymerized glyoxal, in the presence of substantially 0.02 to 0.5 percent of a water-soluble cationic wetting agent consisting of a condensation product of a water-insoluble long-chain fatty acid and an ethanolamine.

PAUL B. DAVIDSON.